

July 15, 1969

C. L. MANTELL ET AL

3,455,799

## ELECTROWINNING MANGANESE

Filed Oct. 19, 1965

2 Sheets-Sheet 1



FIG. I.



FIG. 2.

INVENTORS  
C. L. Mantell &  
G. R. Ferment

BY Harry Brumley

**ATTORNEYS**

July 15, 1969

C. L. MANTELL ET AL

3,455,799

ELECTROWINNING MANGANESE

Filed Oct. 19, 1965

2 Sheets-Sheet 2



FIG. 3.



FIG. 4.

INVENTOR  
C. L. Mantell &  
G. R. Ferment

BY

*Harvey Rommel*

ATTORNEYS

3,455,799

## ELECTROWINNING MANGANESE

Charles L. Mantell, Manhasset, N.Y., and George R. Ferment, Parsippany, N.J., assignors to The Board of Trustees of Schools for Industrial Education of Newark, N.J., administering Newark College of Engineering, Newark, N.J., a public corporation of New Jersey

Filed Oct. 19, 1965, Ser. No. 497,935  
Int. Cl. C22d 1/24

U.S. CL. 204—105

6 Claims

### ABSTRACT OF THE DISCLOSURE

In the electrowinning of manganese zinc ions are added to a catholyte in a manganese deposition cell to reduce the current density necessary to produce pure manganese.

The present invention relates generally to electrowinning manganese and more particularly to a process wherein zinc is added to the catholyte in a manganese deposition cell to reduce the current density necessary to achieve manganese electrolytically.

The production of pure manganese (99.9+%) by electrolysis requires very pure manganese to be in a solution that is fed to the electrolytic cell. If the impurities that usually accompany manganese ore, such as cobalt, nickel, molybdenum and copper are present to any great extent, manganese can not be deposited on the cathode of an electrolytic cell. Actually, the significant presence of any of these impurities causes whatever manganese that is plated on the cathode to recede from it, i.e. go back into solution. Even in the total absence of these impurities the cell must be operated at or above a minimum current density and minimum voltage to achieve manganese deposition. With the addition of the specified impurities even in trace amounts, the current density required for deposition is substantially increased and is accompanied by a slight increase in the voltage necessary for deposition. Hence, to provide the most efficient method of obtaining manganese, i.e. the method requiring minimum current density and minimum voltage for deposition, it has always previously been thought that the catholyte feed to the electrolytic cell must be as free as possible of all metallic impurities.

We have found, unexpectedly and through experimentation, that the addition of trace amounts of zinc to the catholyte actually enhances the deposition of manganese, both in pure solutions and in solutions having trace amounts of the impurities usually accompanying the raw ore. The addition of zinc, in trace amounts, reduces the minimum current density required for manganese to be deposited on the cathode, both when the catholyte solution is pure and when it contains impurities. This result occurs since it has been found that zinc actually aids in the deposition of manganese at the cathode of the cell. Hence, the present invention enables input requirements of the deposition cell to be reduced, whereby increased operating efficiency is achieved. It is also expected that certain ores can be processed without having a filter to remove the usual impurities that accompany manganese ore, such as cobalt, nickel, molybdenum and copper. In addition, the present invention enables deposition to occur at a higher rate than previously if the cell is operated at the same current density.

It is, accordingly, an object of the present invention to provide a new and improved method for electrowinning manganese, which method is more efficient in the use of electric power than prior methods and thereby less expensive in operation.

Another object of the invention is to provide a method

of electrowinning manganese by lowering the minimum current density required for deposition.

Another object of the invention is to provide an electrolytic cell having a catholyte that enables manganese to be deposited at lower current densities than with prior art cells.

A further object of the invention is to provide a method of reducing the power input requirements for the electrolytic fabrication of pure manganese by adding trace amounts of zinc to the catholyte feed to the cell.

An additional object of the invention is to provide a method of electrolytically manufacturing pure manganese wherein the deleterious effects, on the deposition process, of trace amounts of the impurities that accompany the manganese ore are overcome.

Still an additional object of the invention is to provide a method of electrowinning manganese from certain ores without the necessity for precipitating and filtering trace impurities from them.

Yet a further object of the invention is to provide a new and improved method for electrowinning manganese at a higher efficiency than previously possible with the same input power.

The above and still further objects, features and advantages of the present invention will become apparent upon consideration of the following detailed description of one specific embodiment thereof, especially when taken in conjunction with the accompanying drawings, wherein:

FIGURE 1 is a schematic diagram of a typical manganese cell with which the present invention is adapted to be utilized;

FIGURES 2 and 3 are graphs of current density versus voltage for different catholyte solutions applied to the cell of FIGURE 1; and

FIGURE 4 is a plot of current density required for manganese deposition versus zinc concentration in the catholyte.

Reference is now made to FIGURE 1 of the drawings wherein electrolytic cell 11 is divided into anolyte chamber 12 and a catholyte chamber 13 by diaphragm 14 which may be canvas or any other suitable liquid permeable material. Chambers 12 and 13 communicate with each other by overflow pipe 15 that enables the catholyte liquid from chamber 12 to flow into chamber 13.

Variable D.C. potential source 16 is connected between stainless steel cathode 17, located in catholyte chamber 12, and lead alloy anode 18, located in chamber 13, to polarize the anode positively relative to the cathode.

The catholyte in chamber 12 is a solution of the usual concentration of approximately 35 grams per liter of ionic manganese ( $Mn^{++}$ ), approximately 120 grams per liter of ammonium sulphate  $[(NH_4)_2SO_4]$  and approximately 0.1 gram per liter sulphur dioxide ( $SO_2$ ), to which is added trace amounts of ionic zinc ( $Zn^{++}$ ) in concentrations of between 0.15 to 5.0 milligrams per liter. While the maximum zinc concentration can be several times the amount stated, the addition of zinc above a concentration of 5.0 milligrams per liter is wasteful. The temperature of the catholyte solution is approximately 30° centigrade and the pH thereof is about 7.20. The anolyte in chamber 13 is the usual solution of approximately 15 grams per liter of manganese sulphate, 30 grams per liter of sulphuric acid, and approximately 130 grams per liter of ammonium sulphate. The anolyte has a pH of between 1.2 and 1.6.

Anolyte is continuously drawn from chamber 13 by pump 19 that feeds the liquid solution through filter 21 to leaching tank 22. In tank 22, manganese ore, in the form of conditioned manganese oxide ( $MnO$ ), is treated with the filtered anolyte and a leaching solution of am-

monium sulphate and sulphuric acid. The solution emerging from tank 22 is passed through filter 23 which removes metallic impurities that are usually present in the manganese ore and which have not previously been withdrawn from the manganese oxide applied to leaching tank 22. Typical of the impurities that are sometimes withdrawn are: iron, arsenic, antimony, tin, lead, nickel, cobalt, molybdenum, silica, aluminum, calcium and magnesium, although cobalt, nickel, molybdenum and copper are the only impurities present usually to an extent that will cause detrimental results to occur in the manganese deposition. In any event, it is to be noted that zinc is not an impurity found in manganese ores.

Downstream of filter 23, pure zinc is added to the catholyte feed solution in trace quantities so that the catholyte solution in chamber 12 has a concentration of  $Zn^{++}$  ions between 0.15 milligram per liter and 5.0 milligrams per liter. If the upper limit is exceeded, the manganese deposited on cathode 17 does not achieve the 99.9% purity expected from electrolytic processing. Zinc is shown as being introduced into the system downstream of filter 23 because it is difficult, with certain types of filters, to separate it from the natural impurities accompanying the manganese ore. It is to be understood that zinc may, however, be introduced into the system upstream of filter 23 if suitable filters are available. After zinc, in suitable quantities, has been added to the catholyte feed solution, the solution is fed into chamber 12 by pump 24.

To operate cell 11 in the most efficient manner possible, it is necessary to monitor the current density therein, as feed to the cell by source 16, in addition to the polarization voltage of cathode 17 relative to the negative terminal of the source. Current density is measured by connecting D.C. ammeter 24 in series with source 16 and one of the cell electrodes, preferably anode 18 so that the cathode polarization voltage can be more accurately measured. Since the area of electrode 17 is constant, the reading of meter 24 derives a direct indication of cathode current density. The current feed to cell 11 by source 16 and the cathode polarization voltage must be monitored so that the cell can be operated at current densities and polarization voltages above the minimum values required to initiate and maintain manganese deposition on cathode 17.

The polarization voltage is monitored by connecting salt bridge 25 to a portion of cathode 17 that is always submerged in the catholyte. Connected in series with salt bridge 25 is saturated calomel electrode 26 that includes a fiber junction. Electrode 26 is utilized as a reference electrode for measuring the voltage of cathode 17. Standard cell 27, having a voltage on the order of 1.018 volts, is connected between the electrode 26 and voltmeter 28 to buck the voltage from the saturated calomel electrode. With this arrangement, the net voltage drop across the measuring circuit is minimized, whereby current flow through it is virtually zero and accurate measurements are derived without taking significant power from source 16.

To provide an understanding of the operation and advantages of the present invention, reference is now made to FIGURES 2-4. In FIGURES 2 and 3, current density in catholyte chamber 12 is plotted against cathode polarization voltage, i.e. the voltage between the negative terminal of source 16 and salt bridge 25.

Curve 31, FIGURE 2, is a plot of current density versus polarization voltage when the system operation is such that filter 23 has functioned perfectly, whereby no impurities are in the catholyte feed and no zinc has been introduced therein. Under these conditions, deposition of manganese occurs only on the portion of curve 31 at point 32 and to the right thereof, along line 33. If the cathode polarization voltage is less than 1.4 volts and the current density of the catholyte in chamber 12 is less than approximately 135 millamps per square inch, manganese can not be deposited on cathode 17. It is to be noted that both the current and voltage parameters must be reached and maintained for deposition to occur; if only one of these

parameters prevails, manganese will not be coated onto cathode 17. Instead, manganese will recede from cathode 17 into the catholyte solution and thereby nullify the energy previously used for deposition.

Since the voltage required to deposit manganese is substantially fixed by the electrolyte that must be employed, the present invention seeks to decrease the input current required for manganese deposition and thereby increase the efficient use of the electric power supplied to the system by source 16. Decreases in the current density required for deposition have been found to occur if trace amounts of  $Zn^{++}$  ions are added to the catholyte. The decreased current densities required for deposition are illustrated by curves 34-37, FIGURE 2, wherein the concentrations of  $Zn^{++}$  ions in the catholyte are respectively 0.31 milligram per liter, 0.63 milligram per liter, 5.00 milligrams per liter and 15 milligrams per liter. It is noted that the minimum current densities required for deposition, i.e. the points where curves 34-37 intersect line 33, are approximately 110 millamps per square inch, 100 millamps per square inch, 90 millamps per square inch and 85 millamps per square inch, respectively for the four different concentrations. These results are also reflected in the curve of FIGURE 4. Hence, the minimum current densities required for manganese deposition are reduced almost in one-half from 145 millamps per square inch to approximately 85 millamps per square inch by adding trace amounts of  $Zn^{++}$  ions to the catholyte solution and increased operating efficiency is thereby attained.

Another advantage occurring from the addition of trace amounts of zinc to the catholyte is that for a specified current density deposition occurs at a more rapid rate than if zinc had not been added, provided the minimum voltage and current density requirements are met. This is ascertained from the straight lined portion 33 of FIGURE 2 since deposition rate is a function of distance along line 33 from the point at which the line intersects curves 31 and 34-37.

The farther from the intersection point along line 33 one moves, the more rapid the deposition rate becomes. Hence, at point 32, the current and voltage are such that the tendency of manganese to recede from cathode 17 is just overcome and deposition occurs at a slow rate when no zinc has been added to the catholyte solution. In contrast, point 32 is significantly removed from the intersection of curves 34-37 with line 33, evidence indicating that deposition occurs more rapidly when  $Zn^{++}$  ions are added to the solution. Hence, for the same input power necessary to operate the cell at point 32 considerably greater amounts of manganese are deposited during the same interval with the addition of zinc.

It is also interesting to note the beneficial results that the addition of zinc has in compensating for the detrimental effects of the impurities usually found in manganese ore. These detrimental effects can be ascertained from polarization curves 41 and 42, FIGURE 3. Curve 41 is a plot of catholyte current density versus cathode polarization potential when the catholyte contains no impurities. In contrast, curve 42 indicates how much more current is required to achieve manganese deposition when 1.60 milligrams per liter of nickel ions ( $Ni^{++}$ ) are added to the catholyte. Also, curves 41 and 42 provide an indication, by the significant area between them, of the considerably greater power required to bring cell 11 from its rest condition of zero polarization voltage and zero current, when a trace amount of nickel is added.

The adverse effects of the nickel impurity can be compensated and even overcome by the addition of sufficient quantities of zinc. This is indicated by curves 43-45, wherein  $Ni^{++}$  ion concentration is maintained substantially constant at 2.00 milligrams per liter, 2.50 milligrams per liter and 5.00 milligrams per liter, respectively.

Similar advantageous results were found to exist when trace amounts of  $Zn^{++}$  ions were introduced into cath-

olytes containing trace amounts of cobalt ions ( $Co^{++}$ ), copper ions ( $Cu^{++}$ ), and cadmium ions ( $Cd^{++}$ ), as indicated by the following table.

TABLE

| Additive to pure electrolyte | Concentration, mg./L. | Minimum Deposition current, ma./sq. in. |
|------------------------------|-----------------------|-----------------------------------------|
| 1. $Co^{++}$                 | 0.527                 | 371                                     |
| 2. $Co^{++}$                 | 0.527                 | 155                                     |
| 3. $Zn^{++}$                 | 0.63                  |                                         |
| 4. $Cu^{++}$                 | 4.93                  | 178                                     |
| 4. $Cu^{++}$                 | 4.93                  | 145                                     |
| 5. $Zn^{++}$                 | 0.63                  |                                         |
| 5. $Cd^{++}$                 | 5.0                   | 140                                     |
| 6. $Cd^{++}$                 | 5.0                   | 119                                     |
| 7. $Zn^{++}$                 | 0.63                  |                                         |
| 7. $Cd^{++}$                 | 100                   | 152                                     |
| 8. $Cd^{++}$                 | 100                   | 142                                     |
| 8. $Zn^{++}$                 | 0.63                  |                                         |

The tabulated results, indicated by the table and FIGURE 3, show that with the addition of trace amounts of zinc, according to the present invention, the use of certain ores having low impurity content enables filter 23 to be eliminated completely.

While we have described and illustrated one specific embodiment of our invention, it will be clear that variations of the details of construction which are specifically illustrated and described may be made without departing from the true spirit and scope of the invention as defined in the appended claims.

We claim:

1. In the process of electrowinning manganese in an electrolytic cell having a cathode in a catholyte and an anode in an anolyte, said catholyte and anolyte including manganese sulfate and ammonium sulfate, comprising the steps of applying sufficient D.C. power to said cathode and anode to maintain the anode-cathode polarization voltage and cathode current density at least at predetermined levels required to initiate and maintain the deposition of manganese on the cathode, adding trace amounts of zinc ions to a solution including manganese ions, and feeding the solution including the zinc and manganese ions to the catholyte while said voltage and current density

are maintained at least at said predetermined levels said trace amounts of zinc ions being of sufficient quantity to reduce the minimum current density at which manganese deposition occurs on the cathode while the minimum polarization voltage for deposition remains constant.

2. The process of claim 1 wherein said trace amounts of zinc are sufficient to provide an ionic zinc concentration in excess of 0.15 milligram per liter in the catholyte.

3. The process of claim 1 wherein the amount of zinc added is such that the concentration of ionic zinc in the catholyte is between 0.15 milligram per liter and 5.0 milligrams per liter.

4. The process of claim 1 wherein the solution includes trace amounts of cobalt and/or nickel which normally raise the minimum current density required for manganese deposition and the quantity of zinc ions in the solution is sufficient to compensate for the rise in minimum current density required for deposition.

5. The process of claim 4 wherein said trace amounts of zinc are sufficient to provide an ionic zinc concentration in excess of 0.15 milligram per liter in the catholyte.

6. The process of claim 4 wherein the amount of zinc added is such that the concentration of ionic zinc in the catholyte is between 0.15 milligram per liter and 5.0 milligrams per liter.

#### References Cited

##### UNITED STATES PATENTS

- 30 Re. 23,332 1/1951 Ambrose \_\_\_\_\_ 204—105  
2,852,455 9/1958 Hausner \_\_\_\_\_ 204—151  
2,863,813 12/1958 Juda et al. \_\_\_\_\_ 204—180

##### OTHER REFERENCES

- 35 Schlain et al., Effect of Impurities on the Electrodeposition of Manganese, Bureau of Mines, Report of Investigations, May 1946, U.S. Dept. of the Interior.

JOHN H. MACK, Primary Examiner

40 H. M. FLOURNOY, Assistant Examiner